

1

3,796,679

## ADHESIVE COMPOSITION

Erich F. Kujas, Philadelphia, Pa., assignor to Prodesco, Inc., Parkasie, Pa.

No Drawing. Continuation-in-part of application Ser. No. 864,205, Oct. 6, 1969, now Patent No. 3,645,951. This application Feb. 9, 1972, Ser. No. 224,952.

The portion of the term of the patent subsequent to Feb. 29, 1989, has been disclaimed

Int. Cl. C08g 51/24

U.S. CL. 260—29.4 UA

15 Claims

## ABSTRACT OF THE DISCLOSURE

An adhesive composition and method of making such composition are disclosed. The composition is suitable for use in bonding carpeting yarns to carpet backing. The composition consists essentially of hydroxy methacrylic acid ester latex, a melamine formaldehyde condensate, dodecetyl succinic anhydride and zinc oxide.

This application is a continuation-in-part of copending application, Ser. No. 864,205, filed Oct. 6, 1969, now U.S. Pat. No. 3,645,951.

## BACKGROUND OF THE INVENTION

In the manufacture of tufted carpeting, yarns of a textile fibrous material, which may be of natural origin such as wool, mohair, cotton, etc., or a synthetic fiber such as a polyamide, viscose rayon, polyesters, polyacrylonitrile or the like, are pushed through a fabric backing such as a non-woven fabric or a woven fabric as, for example, burlap or cotton. An adhesive is applied to the yarn loops which are in contact with the back side or ultimate bottom of the carpet to bond the yarns to the backing. A secondary backing, which may also be a woven or non-woven fabric or foamed latex backing such as shown in U.S. Pat. 3,215,647, may then be placed over the loops and primary backing. If the secondary backing is sufficiently open, the adhesive may be applied after the secondary backing is in place. Otherwise, the secondary backing is placed over the wet adhesive which has been previously applied to the primary backing and yarn loops. The yarns which are on the front or ultimate top side of the carpet are frequently cut and are thus bonded in place by the described adhesive. If a secondary backing is also used, the adhesive likewise, of course, holds such backing in place.

Adhesives previously available for the bonding of carpet yarns to a carpet backing having generally been based on a natural or synthetic latex, as, for example, that disclosed in U.S. Pat. 2,748,446. Such compositions, however, have possessed several limitations. In the first place, the adhesives do not wet and penetrate the backing and yarns to a sufficient extent to provide a firm and stable bond. Subsequent cleaning, which involves the use of water and/or detergents, causes rapid deterioration of the limited bond, which results in the yarns (including individual plies in a multiple yarn) or individual fibers or filaments thereof being easily pulled from the backing. This has been found to be a particularly severe situation with yarns of fibrous materials such as mohair, nylon, polyesters and acrylics, which do not have scaled surfaces or which are not crimped.

Moreover, piece dyeing of carpeting made with such

2

adhesives, which involves hot or boiling aqueous dye solutions, causes rapid deterioration of the adhesive bond, also adhesive compositions, even after curing, often contain components which leach out into the dye bath, which has deleterious results such as causing uneven dyeing, particularly with certain synthetic yarns. Also, the adhesives often do not cure well or rapidly at elevated temperatures and coagulate to tacky accumulations which requires one or two additional passes through the curing oven or even standing overnight to complete the cure. Another very serious limitation of such adhesives has been found to be poor shelf life in the container, the adhesive gelling in relatively short periods of time.

This is especially important, since it is quite advantageous in the manufacture of carpet to utilize containers capable of holding large quantities of the adhesive which can be used over an extended period of time. In addition to the foregoing limitations, adhesive compositions previously available for the specified use have been susceptible to relatively rapid surface hardening upon exposure to the atmosphere and also poor flexibility after curing.

## SUMMARY OF THE INVENTION

The present invention is thus directed to an adhesive composition and method of making the same, which composition is not susceptible to the foregoing disadvantages. The composition consists essentially of a hydroxy acrylic acid ester latex, a melamine formaldehyde condensate, dodecetyl succinic anhydride and zinc oxide in specified proportions. The hydroxy acrylic acid ester latex is used in a quantity of from about 45 to about 90 parts by weight of acrylic latex solids, while from about 1 to about 2.5 parts by weight of the melamine condensate, 0.5 to about 2 parts by weight of the anhydride and from about 6 to about 15 parts by weight of zinc oxide, preferably from about 6 to about 12 parts by weight, are used. The composition may also include about 1 part by weight of calcium hydroxide and/or magnesium hydroxide as a filler. The composition has a pH within the range of from about 6 to about 7, with a pH of from about 6.1 to about 6.8 being preferred.

The adhesive composition is preferably prepared as follows. The melamine formaldehyde condensate and the dodecetyl succinic anhydride are first mixed at a temperature of from about 100 to about 120° F. The resulting mixture is then mixed with the hydroxy acrylic acid ester latex at a temperature of from about 100 to about 130° F. To the resulting mixture is then mixed the zinc oxide (dry), and, at about the same time, the calcium and/or magnesium hydroxide, if used, at a temperature of from about 100 to about 140° F. The final mixture is at from about 100 to about 140° F. to provide complete blending. The composition may then be cooled to room temperature and stored for ultimate use or it may be used immediately.

One of the principal components of the present adhesive composition is a hydroxy acrylic latex. This is essentially a high solids content (about 50%) emulsion of a poly hydroxy acrylic (including methacrylic) acid ester. The preferred material is a poly hydroxyalkylmethacrylate in which the alkyl group contains 2 to 3 carbon atoms, namely, poly hydroxyethylmethacrylate and poly hydroxylpropylmethacrylate.

The second important component of the present adhesive is the melamine formaldehyde condensate. The

preferred material in this regard is essentially methylol melamine formed by condensing one mol of formaldehyde with one mol of melamine. The melamine formaldehyde condensate is believed to react with the hydroxyacrylic acid ester polymer causing crosslinking on curing.

However, the advantageous characteristics of the present adhesive depend upon the inclusion of the dodecetyl succinic anhydride and the zinc oxide in the stated proportions. The former, which is a liquid compatible with the other components, provides functional groups enhancing crosslinking of the acrylic latex on curing, imparting flexibility, high temperature resistance and detergent and water resistance to the cured adhesive. In addition, the dodecetyl succinic anhydride alters the viscosity of the composition causing it better to wet and penetrate yarns and backing evenly, without bleeding out of the top side of the backing, and imparts long shelf life to the adhesive. The zinc oxide stabilizes the composition, including its viscosity as a function of the composition's pH and serves as a curing promoter.

The inclusion of calcium hydroxide and/or magnesium hydroxide is particularly advantageous as a filler to control and adjust the pH of the composition and hence its viscosity. Calcium hydroxide is preferred.

The following is a specific example of the adhesive composition of the present invention and its preparation: with 2.5 parts, by weight, of melamine formaldehyde condensate, essentially methylol melamine (in the form of a high viscosity liquid containing 80% solids and providing 2 parts of melamine formaldehyde condensate solids) are mixed 2 parts, by weight, of dodecetyl succinic anhydride, at 120° F. The resulting mixture is then added to and mixed with 180 parts, by weight, of hydroxy acrylic latex (essentially poly hydroxyethylmethacrylate, 50% solids, providing 90 parts, by weight, of solids), at 125° F. There are then added 12 parts, by weight, of zinc oxide (oven dried) and 1 part of calcium hydroxide, and the total is heated, while mixing, at 140° F. The resulting adhesive has a pH of about 6.2. Poly hydroxypropylmethacrylate latex may be used to replace some or all of the poly hydroxyethylmethacrylate.

The adhesive composition of the present invention has an excellent shelf life, having stood in a closed container for 3 months without any apparent change. Moreover, it has been cooled in a refrigerator without the deleterious results often noted with other latex compositions. When applied to yarn loops and adjacent backing, it readily wets them penetrating into the yarns and the backing without, however, bleeding through deleteriously to the front or ultimate top side of the carpeting. On heating to from about 215 to about 300° F. for curing, the adhesive cures completely and evenly in 1-2 minutes depending upon the temperature. Curing the adhesive at elevated temperatures does not result in discoloration thereof ("staining") as has been found to be the case with most other latex adhesives. Carpeting made using the present adhesive can be, in the cured or partially cured conditions, subjected to piece dyeing (the heat encountered during piece dyeing and setting being relied upon to complete the cure, if necessary) without weakening the bond, causing deterioration of the adhesive or loss of fiber into the dye bath. Moreover, the composition is compatible with other aspects of carpet manufacture; for example, nothing leaches from the adhesive into the piece dye bath to contaminate the latter. The cured adhesive is flexible and resilient and is not adversely affected by detergent solutions commonly used in cleaning (shampooing) carpeting. It has also been found to be fire resistant according to AATCC test methods 33-1962 and 34-1966. The cured adhesive has a high degree of porosity and exhibits good affinity for dyestuffs normally used in piece dyeing carpeting; hence very little or no adhesive can be seen as such after piece dyeing, depending upon the particular dyestuff and yarn. Tufted carpeting made of smooth fibers, utilizing

the present adhesive, has been subjected to piece dyeing and to cleaning with detergent solutions, and the yarns and individual fibers thereof have remained locked in place by the adhesive bond.

Although further illustrative examples of the adhesive composition, utilizing other quantities of the various components within the specified ranges, could be recited herein, such examples are not necessary for an adequate understanding of the invention. Accordingly, for the sake of brevity of disclosure, no additional examples will be set forth. It should also be understood that one preferred composition contains approximately 90 parts by weight of the described acrylic acid ester solids, about 2 parts by weight melamine formaldehyde condensate, about 2 parts by weight dodecetyl succinic anhydride, about 12 parts by weight zinc oxide, and optionally about 1 part by weight of calcium hydroxide and/or magnesium hydroxide, with the pH being within the previously indicated preferred range of about 6.1 to about 6.8, to provide a composition possessing highly satisfactory stability and viscosity characteristics.

I claim:

1. An adhesive composition for use in bonding carpeting yarns to carpet backing consisting essentially of from about 45 to about 90 parts by weight of polyhydroxy alkylmethacrylic acid ester latex solids, about 1 to about 2.5 parts by weight of a melamine formaldehyde condensate, about 0.5 to about 2 parts dodecetyl succinic anhydride, and from about 6 to about 15 parts by weight zinc oxide.
2. The composition of claim 1 in which said composition has a pH of from about 6 to about 7.
3. The composition of claim 2 in which said composition has a pH of about 6.1 to about 6.8.
4. The composition of claim 1 including about 1 part by weight of calcium hydroxide and/or magnesium hydroxide.
5. The composition of claim 1 wherein said poly hydroxyalkylmethacrylic acid ester latex contains 2 to 3 carbon atoms in the alkyl group.
6. The composition of claim 1 in which said melamine formaldehyde condensate is methylol melamine.
7. The composition of claim 5 in which said melamine formaldehyde condensate is methylol melamine.
8. The composition of claim 7 including about 1 part by weight of calcium hydroxide and/or magnesium hydroxide.
9. An adhesive composition for use in bonding carpeting yarns to carpet backing consisting essentially of from about 45 to about 90 parts by weight of polyhydroxy alkyl methacrylic acid ester latex solids, about 1 to about 2.5 parts by weight of a melamine formaldehyde condensate, about 0.5 to about 2 parts by weight of dodecetyl succinic anhydride, and from about 6 to about 15 parts by weight of zinc oxide, said composition having a pH of from about 6 to about 7, said latex being a poly hydroxyalkylmethacrylate in which the alkyl group contains 2 to 3 carbon atoms and said melamine formaldehyde condensate is methylol melamine.
10. The composition of claim 9 in which said composition has a pH from about 6.1 to about 6.8.
11. The composition of claim 10 in which said zinc oxide is present in a quantity of from about 6 to about 12 parts by weight.
12. The composition of claim 11 including about 1 part by weight of calcium hydroxide and/or magnesium hydroxide.
13. A method of making an adhesive composition suitable for bonding carpeting yarns to carpet backing which comprises mixing about 0.5 to about 2 parts by weight of dodecetyl succinic anhydride with about 1 to about 2.5 parts by weight of a melamine formaldehyde condensate at a temperature of from about 100 to about 120° F., admixing the resulting mixture with from about 45 to about 90 parts by weight of polyhydroxy alkyl methacrylic acid ester latex solids at a tem-

perature of from about 100 to about 130° F., and subsequently mixing about 6 to about 15 parts by weight of zinc oxide with the resulting mixture at a temperature of from about 100 to about 140° F.

14. The method of claim 13 in which about 1 part by weight of calcium hydroxide and/or magnesium hydroxide is mixed with said mixture at about the same time said zinc oxide is admixed therewith.

15. The composition of claim 1 in which said zinc oxide is present in a quantity of from about 6 to about 12 parts by weight.

## References Cited

## UNITED STATES PATENTS

3,645,951 2/1972 Kujas ----- 260—29.4 U A

5 LORENZO B. HAYES, Primary Examiner

U.S. Cl. X.R.

260—39 R, 41 B, 856